

Patented July 11, 1933

1,917,938

*Biocidal*

## UNITED STATES PATENT OFFICE

STUART JACKSON HAYES, OF LUDLOW, MASSACHUSETTS, ASSIGNOR TO LUDLOW MANUFACTURING ASSOCIATES, OF LUDLOW, MASSACHUSETTS, A MASSACHUSETTS TRUST

## THREAD

No Drawing.

Application filed October 14, 1931. Serial No. 568,875.

This invention relates to improvements in yarns and threads used in the manufacture of fish nets, more particularly gill nets. It includes both the method of preserving such 5 yarns and threads so as to make them rot-resistant and the rot-resistant yarns and threads themselves.

The rapid deterioration and resulting replacement costs of fishing nets has resulted 10 in efforts to find a satisfactory preservative treatment. A great deal of work has been done by the United States Bureau of Fisheries on the problem and the results have been described in bulletins of that bureau. So far 15 as I am aware all suggestions for preserving nets refer to the treatment of the finished fabric.

The various substances which have been suggested for treating such nets, so far as I 20 am aware, include only substances which can be used for treating the finished fabric, and do not include substances suited for treating the thread prior to the fabrication of the netting. When applied to the thread many 25 preservative substances applicable to completed nets produce one or another of several desirable effects which render the thread unsuitable for subsequent use in the manufacture of the nets. Tar, for example, has been 30 used as a preservative but it stiffens the nets. If applied to thread the thread would be too stiff to be passed through the knitting machine. Copper oleate has been suggested but this would also render the thread too stiff for 35 subsequent use. Other substances change the character of the thread in such a way that it is not suitable for knotting. So far as I am aware there have been no rot-resistant threads on the market suitable for the production of fish nets, more particularly gill 40 nets.

According to this invention, flax yarn or thread is made rot-resistant by a process which leaves the thread soft and pliable and 45 with a surface and composition suited to knotting. According to a preferred method of treatment, both a disinfectant and a water-proofing material are applied to the thread. One or both of these ingredients 50 may be applied to the thread after it is man-

ufactured, or they may be applied to the yarn before or during the manufacture of the thread or they may be applied in part during the manufacture and in part after the completion of the thread.

It is often advantageous to treat the thread before it is made up into netting, not only because of the reduced cost of preserving the net in this way rather than by applying the preservative to the finished net, but also because treatment before the thread is manufactured into the net insures more uniform and more thorough treatment of the thread. The thread in a net is not under uniform tension. Parts of the thread, as at the knots, 60 are under greater tension than other parts. The tight parts absorb liquors less readily. Furthermore, the interior of the knots is protected and may not be as thoroughly or uniformly impregnated when preservatives are 65 applied to the finished netting. By applying the preservative to the thread before it is fabricated into the netting, uniform treatment of the thread is insured.

I find it of advantage to apply to the 70 yarn or thread a disinfectant which is only slightly soluble in water. When water-proofed the disinfectant does not readily wash away and will remain on or in the threads in effective quantities for a long 75 period of time, usually until the net fails by natural wear and tear, although in some instances further applications of the preservative treatment may be made before the end 80 of the effective life of the net.

According to a preferred method of treatment I apply disinfectants which of themselves would not remain on the fiber in sufficient concentration for the required length 85 of time but which nevertheless would be effective disinfectants for preventing or retarding the growth of micro-organisms, or destruction or rotting of the fibers thereby when applied in connection with a water-proofing material. A disinfectant which I have found 90 particularly valuable is thymol. Other disinfectants, particularly phenolic substances of limited solubility but effective disinfecting 95 action such as salicyl anilide, phenyl salicylate, sodium phenate, hexylresorcinol and 100

some other higher alkyl resorcinols can be employed. The amount of the disinfectant employed will vary somewhat with the disinfectants, but should be sufficient to protect 5 the netting against objectionable deterioration or rotting.

The water-proofing substances employed in connection with the disinfectant are substances which impart water-resistance to the fibers without objectionable stiffening of the fibers. I consider metallic soaps such as 10 aluminum soap particularly advantageous. Soaps of lead, iron, etc. can be employed, but I consider them less desirable than aluminum 15 soap because the soaps of these other metals impart dark colors and are heavy. The soaps may be soaps of the common fatty acids such as oleates, stearates, palmitates, etc. or soaps of resin acids, etc. The amount of water- 20 proofing agent employed should be sufficient to impart water-resistant or water-repellent properties to the thread, but should not be sufficient to stiffen the thread or deprive it of the desired softness and pliability.

25 In applying the disinfectant and water-proofing compounds it is possible to apply them at the same time and by a single operation. For example, using thymol as the disinfectant and aluminum palmitate as the 30 water-proofing agent, these substances may be dissolved in a suitable solvent such as gasoline and employed for impregnation of the thread followed by wringing and drying.

As an example of this method of treating 35 the thread, one part by weight of thymol is dissolved in 100 parts by weight of gasoline with stirring until solution takes place and two parts by weight of aluminum palmitate are added and the mixture stirred until the 40 soap is dissolved or dispersed. The resulting dispersion looks like a perfect solution until it is allowed to settle when it sets as a rather viscous fluid with a thickness comparable to that of molasses but not sticky. The thread 45 reeled into hanks is immersed in this material and then after removing the excess of liquid it is passed through a wringer and then allowed to dry by evaporation of the gasoline. If 100% by weight of the immersion fluid is 50 left on the thread about one-half percent by weight of thymol and one percent by weight of aluminum palmitate will be left on the thread after drying.

Instead of combining the application of 55 the disinfectants and the water-proofing agents, it is often preferable to carry out the operation in two stages. This can be done to advantage by first applying a soluble soap and the disinfectant to the yarn 60 during the manufacture of the thread and then subsequently treating the impregnated fiber with an aluminum salt solution, after completion of the thread, to precipitate the insoluble aluminum soap in the fiber. In 65 this way a protective layer of the aluminum

soap is developed from the soluble soap after the thymol has been applied under intimate dispersion and suspension in the soluble soap solution and the treatment is advantageously effected in conjunction with other wet treatments of the yarn or thread, thus avoiding any additional drying costs.

This preferred method of treating the threads may be carried out in accordance 70 with the following specific example: a 10% solution in water of an ordinary chipped soap such as the fatty oil soaps used by dyers is, allowed to cool to about 50° C. 5% of finely powdered thymol is added with stirring until the thymol is melted. The thymol rises to the top of the soap dispersion and forms an oily layer. When the mixture is 75 nearly cooled but before the thymol crystallizes it is stirred violently for a few minutes until a creamy colloidal suspension is obtained which can be diluted to the equivalent of about 2% soap concentration for use in the impregnation. This dilution can be carried out satisfactorily in hot water but not in 80 cold water. A faintly opalescent liquid results.

This suspension or solution is advantageously applied to the yarn in the following manner: Flax yarn such as that ordinarily used for gill nettings is thoroughly boiled and after drying the yarn is wet-twisted through the soap suspension of thymol and then dried at temperatures which will not drive off the thymol. The twisted thread is 90 then dipped into a cold aqueous solution of aluminum acetate of about 1.025 specific gravity, and dried and spooled. The treated thread may then be made up into nets directly, or it may be shipped to a netting manufacturer. The water soluble soap provides a vehicle for distributing the solid thymol in a finely divided precipitated form on and in the fiber and when combined by reaction with the aluminum or other metal produces in situ a metallic soap. This metallic soap is not only on but within the fiber substance itself and is effective as a water- 95 proofing agent and holds the disinfectant on the fibers in a concentration such that it retains its protective action over a long period of time.

The thread thus treated is uniformly impregnated with the preservative throughout its entire length and the netting made from it is uniformly impregnated within the knots and at those portions of the netting which are under high tension as well as those portions which are under slight tension or no tension. The netting contains an effective disinfectant. This rot-resistant netting is 100 soft and pliable. It flattens when struck by fish and is in every way suitable for gill netting.

I claim:

1. The method of preparing a rot-resistant 105

flax thread, which comprises applying a water soluble soap and disinfectant to the yarn, twisting the yarn into thread, and then precipitating the soap within the finished thread 5 by converting it into an insoluble soap.

2. In the method of preparing a rot-resistant flax thread, the steps which comprise impregnating the yarn after boiling with a water soluble soap, twisting the yarn to thread 10 and then converting the soluble soap to an insoluble soap.

3. A rot-resistant flax thread suitable for use in the manufacture of gill netting preserved by the incorporation therein of a 15 solid emulsion of a disinfectant dispersed in an effective waterproofing material.

4. A rot-resistant flax thread suitable for use in the manufacture of gill netting preserved by the incorporation therein of a 20 solid emulsion of thymol dispersed in an insoluble aluminum soap.

5. A rot-resistant thread suitable for use in the manufacture of gill netting, which thread is soft, and pliable and has a surface 25 suitable for knotting, said thread being preserved by the presence therein of a solid emulsion of a difficultly soluble disinfectant dispersed in an effective waterproofing ma-

terial which prevents or retards the dissolving or washing off of the disinfectant.

6. A rot-resistant flax thread suitable for use in the manufacture of gill netting, which thread is soft and pliable and has a surface 70 suitable for knotting, and which thread is preserved by the presence therein of a solid emulsion comprising an insoluble soap with a disinfectant dispersed therein.

7. A rot-resisting flax thread suitable for 75 use in the manufacture of gill netting, which thread is soft and pliable and has a surface suitable for knotting, and which thread is preserved by the presence therein of a solid emulsion of a solid and difficultly soluble disinfectant dispersed in an insoluble aluminum 80 soap.

8. The method of preparing a rot-resistant flax thread which comprises treating the material with a colloidal suspension of a solid and difficultly soluble antiseptic in a water soluble soap and subsequently treating the material with a solution of a metal which will form in situ within and upon the fibers 85 an insoluble soap within which the antiseptic 90 is dispersed as a solid emulsion.

In testimony whereof I affix my signature.  
STUART JACKSON HAYES.

30

95

35

100

40

105

45

110

50

115

55

120

60

125

65

130